

# UNITED STATES PATENT OFFICE.

LEON L. KATZENSTEIN, OF WORCESTER, MASSACHUSETTS, ASSIGNOR TO NORTON COMPANY, A CORPORATION OF MASSACHUSETTS.

## LUBRICATING ABRASIVE WHEEL AND METHOD OF MAKING THE SAME.

1,325,503.

Specification of Letters Patent.

Patented Dec. 16, 1919.

No Drawing.

Application filed December 8, 1917. Serial No. 206,334.

To all whom it may concern:

Be it known that I, LEON L. KATZENSTEIN, a citizen of the United States of America, residing at Worcester, in the county of 5 Worcester and State of Massachusetts, have invented certain new and useful Improvements in Lubricating Abrasive Wheels and Methods of Making the Same, of which the following is a full, clear, and exact specification.

In the art of grinding surfaces by means of abrasive wheels, it is often desirable to fill the pores of a wheel with a suitable lubricant, such as waxes, greases, oils and fats, 15 which is not hardened by heat like a wheel bond, in order to lubricate the wheel and decrease the friction of grinding and therefore decrease the heat generated and the power required during the operation. A 20 lubricant furthermore prevents loading of metal particles in the face of the wheel, because the pores thereof are already partly filled and because the metal being ground does not readily get hot and form soft globules or particles capable of adhering to the 25 walls of the pores. These lubricating fillers also appear to have the property of allowing the abrasive particles to penetrate deeper into the work and therefore cut faster, the 30 greater strain upon the cutting particles causing them to break off more readily and therefore prevent glazing of the face of the wheel.

Wheels filled with such materials have, 35 however, proven unsatisfactory for many types of grinding operations, due to the fact that preferred wheel fillers do not have any large adhesive properties and tend to melt under the heat of grinding and to be constantly thrown centrifugally from the rotating wheel on to the operator and adjacent articles as the wheel wears away. Depending upon the character of the material used, the filler may volatilize under the heat and 45 give off an objectionable odor or smoke, and may even burst into flames. Hence, in certain types of grinding which may involve a considerable evolution of heat, operators often refuse to use a filled wheel, thereby limiting these otherwise satisfactory wheels

to grinding operations which produce only a low heat at the point of contact.

It is accordingly an object of my invention to eliminate the above disadvantages and to provide a self lubricating, non-spattering abrasive wheel of great utility in fields heretofore prohibited because of the detrimental effects noted, and which contains the maximum amount of an easily melted, non-bonding, lubricating filler, capable of making the wheel cooler acting, which will not be centrifugally thrown from the wheel to an objectionable extent under normal grinding conditions. With this and other objects in view, as will appear from the following disclosure, my invention resides in the combination of parts and the steps in a process herein set forth and pointed out in the claims appended hereto.

In filling a previously bonded abrasive 70 wheel with a lubricant, such as paraffin, it has heretofore been customary to heat the wheel to a temperature as high as the melting point of the paraffin, and then dip it, while hot, into a bath of the molten material. Because of the heat-retaining qualities of the abrasive wheel, the paraffin remains melted in the wheel pores into which it has penetrated for some time after the wheel has been removed from the path, and, 75 in accordance with the old method, is drained first from one circular side and then from the other by placing the hot wheel upon a suitable support and reversing it after a few minutes. In this manner, all 80 of the excess filling material which is not held by capillary attraction or by the attraction of the pore walls for the molten material is eliminated. However, an insufficient amount has been removed, since only 85 that force involved in the attraction of gravity has been utilized, while the centrifugal force acting upon the rapidly rotating wheel during grinding is much larger and can easily overcome the attraction of the pore 90 walls for the filler after it has been melted by the heat of grinding. It is accordingly 95 the main purpose of my invention to eliminate this excess filler material which is thrown out centrifugally and to make a lu- 100

briicated abrasive wheel more useful in the art of grinding.

In the practice of my invention, I accordingly incorporate into the pores of a previously bonded abrasive body a lubricating filler in fluid condition, as for example molten or in solution, the filler to be one which is not chemically changed or hardened by heat into an adherent wheel-strengthening bond, but which after solidification will tend to soften under heat and cause the wheel to act softer or will otherwise act to serve as a lubricant and make the wheel cooler acting in the normal grinding operation. For this purpose I may utilize such non-bonding substances as waxes, greases, oils and fats, or mixtures of these with other substances. As a specific illustration, I prefer to use paraffin or paraffin combined with rosin. Since, as above explained, such materials are melted and thrown from the normally rotated wheel, I initially eliminate from the wheel pores substantially all that excess material which would be thrown out centrifugally during grinding, but would ordinarily be retained while fluid against the attraction of gravity. For this purpose I employ a force of sufficient magnitude to counteract the capillary attraction of the pore walls for the filler, and obviously may use various principles or methods of operation. While such means as a jet of steam or gas or a vacuum may be employed, I prefer to use centrifugal force, since it can be easily regulated and conditions readily duplicated, and since it involves similar effects upon the wheel to those caused by rotation during grinding.

As a simplified method of incorporating the right amount of filler in a wheel, I may heat the wheel, as by means of an oven, to a temperature preferably higher than the melting point of the filler to be used,—e. g. paraffin,—and dip the hot wheel into filler previously melted until the pores have taken up the full amount, or as much as is determined by practice to be desirable. The wheel is then mounted upon bearings while hot and while the paraffin is still molten and is rapidly rotated until the centrifugal force generated has eliminated substantially all of that excess of filling material which would be thrown out under the heat of the actual grinding operation, it being obvious that a large proportion of the filler is permitted to remain in the pores.

For example, a pre-heated twelve-inch vitrified aluminum oxid wheel of medium grit and grade may be immersed in molten paraffin until the pores are substantially filled. The wheel is then immediately mounted on an arbor and rotated, before the paraffin has hardened, at a gradually increasing speed until the rate is about 3,000 surface feet per minute, the rotation being

continued for about three minutes. It is found that a wheel treated in this manner may be utilized for grinding at a rate of 5,000 surface feet per minute more or less, depending on the character of the work being ground, without the paraffin spattering from the wheel to any material extent. This rate of rotation employed in removing the excess filler may be considerably less than the normal speed employed in grinding, depending upon the temperature and the fluidity of the filler in the pores, as well as exterior conditions such as the temperature of the room and the character of the work to be ground. While it is desirable to mount the wheel upon bearings in its normal rotating position, it is of course obvious that it may be mounted in any other desired fashion and rotated in any manner by any suitable means.

In accordance with this invention, I eliminate sufficient of the excess filler to make the wheel not only unobjectionable for all ordinary grinding uses but of greatly increased utility in new fields, and I provide therefor a simple and economical manner of filling the wheel to the required amount with sufficient lubricant for all practical purposes and at the same time eliminate the labor and time consumed heretofore in turning the wheels and draining out the excess filler, in accordance with the old practice.

Having thus described my invention, what I claim as new and desire to secure by Letters Patent is:

1. A non-spattering, self-lubricating grinding wheel comprising a porous, coherent body of bonded abrasive material and a lubricating non-bonding filler, capable of readily softening under the heat of grinding and making the wheel cooler acting, which is incorporated in the pores of the body and substantially all of which permanently adheres to the pore walls when subjected to the centrifugal force and heat involved in the normal grinding operation.

2. The method of making a non-spattering, self-lubricating grinding wheel having a porous body of bonded abrasive grain comprising impregnating the pores of the body with a lubricating non-bonding material in fluid condition and then, while said material is fluid, forcibly removing from the pores substantially all of that excess material which, after solidifying, will not be permanently retained within the pores under the centrifugal force and frictional heat generated in a normal grinding operation.

3. The method of making a non-spattering, self-lubricating grinding wheel having a porous, coherent body of abrasive material, comprising heating said wheel body and impregnating the pores thereof with a molten lubricant, maintaining the lubricant in a fluid condition, rotating said body at a

velocity, less than the normal grinding rate for which the wheel is adapted, which will remove substantially all of that excess of lubricant which would not be permanently retained, after solidification, under the centrifugal action and heat generated in the normal grinding operation, maintaining

said rotation until said excess of material has been removed and cooling the wheel body to solidify said lubricant within the wheel 10 pores.

Signed at Pittsburgh, Pennsylvania, this 30th day of November, 1917.

LEON L. KATZENSTEIN.